

Feb. 4, 1947.

E. J. MERRELL

2,415,184

ELECTRIC DEVICE WITH ELECTRON BARRIER

Filed Feb. 5, 1943



$$\text{TIME FACTOR} = 1/12(a/t)^2 + 2/3(a/t - 1)$$

$a$  = RADIUS IN INCHES UNDER LEAD SHEATH

$t$  = THICKNESS OF CONDUCTOR INSULATION IN INCHES

INVENTOR.  
EDWIN JOSEPH MERRELL

BY

  
ATTORNEY

## UNITED STATES PATENT OFFICE

2,415,184

ELECTRIC DEVICE WITH ELECTRON  
BARRIER

Edwin Joseph Merrell, Eastchester, N. Y., assignor  
to Phelps Dodge Copper Products Corporation,  
Dover, Del., a corporation of Delaware

Application February 5, 1943, Serial No. 474,886

2 Claims. (Cl. 174—25)

1

This invention relates to a means for enabling the full electric strength of an insulating medium of an electrical device to be realized, without loss due to local surface weaknesses. Its application is to electric cables, condensers, and insulating windings of other electric devices; more particularly it consists of a sheet of novel material applied to the surfaces of the insulating medium.

The characteristics of this electron barrier are: (1) ability to suppress ionization; (2) high permeability to gases so as to permit thorough and efficient drying of the insulating medium; (3) high permeability to liquids so as to permit thorough and efficient impregnation of the insulating medium; (4) chemical inertness with respect to adjacent materials with and without applied electric stress; (5) absence of gas adsorption so as to preclude the possibility of gas evolution under electric stress.

It is well known that the energy of electrical discharge from metallic conductors into dielectrics may be greatly reduced by interposing, between the metal and dielectric, a layer which possesses high energy absorption characteristics by virtue of high dielectric loss.

I have discovered that this desirable result may be obtained by employing a layer of material which exhibits a high work function, the work function being a measure of the electric energy required to detach electrons. An electron barrier consisting of a layer of material which exhibits a high work function represents a far more efficient means than the former of obtaining the benefits of this electrical phenomenon, because it accomplishes the ionization suppressing function through a low loss impedance rather than through a high loss resistance. The practical effect of such a layer is to suppress or reduce the destructive energy of electric discharges which occur in dielectrics at conductor surfaces, particularly in vacuous pockets, by substantially restricting the charging current of an electric device to a low loss condensive path. This, of course, increases the life of the dielectric, particularly if subjected to occasional over voltages.

Work function is measured in volts, these volts representing the potential level that must be attained to produce electron emission in vacuo. For metals or carbon the value is between 3 and 6 volts, whereas for good insulation, it is substantially infinite up to the breakdown point.

The foregoing and other features of my invention will now be described in connection with the accompanying drawing forming part of this specification in which I have represented an

2

electric device embodying my electron barrier in its preferred form, after which I shall point out in the claims those features which I believe to be new and of my own invention.

5 In the drawing:

Figure 1 is a part section showing my invention as applied to an electric device.

Figure 2 is a graph of a charging current wave of an electric device in which my invention is not used.

Figure 3 is a similar graph of a charging current wave of an electric device in which my invention is used.

Figure 4 is a curve showing how drying time of insulation may be affected by the use of my invention.

15 In the carrying out of my invention I place my electron barrier 11 between the insulation 12 and the conductors 13.

20 While the structure details of the several electric devices in which my electron barrier is employed in the carrying out of my invention vary greatly, the electron barrier is always interposed between the conductor and its associated insulation.

25 For the purposes of this invention an intermediate value of work function, several times as great as that for metals, is required, since the aim is to reduce and equalize electron emission

30 rather than to dam it. Due to experimental difficulties in determining work function in terms of volts, I have adopted a more practical procedure using a cathode ray oscilloscope. Comparing, by this means, the high energy content of discharge

35 from metal with that from my electron barrier, I find the latter is markedly less. Thus the oscilloscopes of Figures 2 and 3 were obtained by photographing the 60 cycle charging current waves, as reproduced by a cathode ray oscilloscope.

40 The oscilloscope shown in Figure 2 is typical of the electric discharge across a gaseous void between a highly conducting metal conductor and a high resistivity, low-power-factor insulation. The oscilloscope shown in Figure 3

45 is similarly typical of the discharge across a gaseous void between a highly conducting metal conductor covered with my electron barrier and the same high resistivity, low-power-factor insulation. It will be noted that, in the construction

50 without the electron barrier, both the peak values and the R. M. S. value of the discharge are many times those characteristic of the design which does possess the electron barrier. The oscilloscope in Figure 2 shows that this type of

55 discharge, not only contains more energy as

shown by the higher R. M. S. value, but also liberates this energy at a much higher intensity, as indicated by the high peaks. It is consequently very much more destructive to surrounding dielectric than the low energy discharges of the type shown in Figure 3.

It is by means of such tests with the cathode ray oscilloscope that I have discovered that sheets consisting largely of submicroscopic silicon carbide, titanium carbide, and titanium carboxide possess electron barrier qualities of a very high order.

A sheet of the above characteristics is particularly valuable for application to high voltage electric devices, the insulation of which in the course of manufacture first must be vacuum treated, then impregnated with low power factor fluid. In manufacturing procedures of this description, every effort must be made to eliminate, or, as much as is practical, reduce impedance to the flow of fluids, gaseous or liquid. Under the high vacuum employed, that is, one millimeter of mercury absolute or less, the gas and moisture which are sorbed in the dielectric assume highly enlarged volumetric dimensions. These quantities of fluid nevertheless must be removed during the manufacturing process in the interest of ultimate operating success for the device; and in the interest of manufacturing economy, this gaseous fluid removal and the subsequent impregnation with liquid insulating fluid must be achieved within a minimum of time.

Impervious electron barriers would not permit attainment of minimum manufacturing time. For example, consider the vacuum drying characteristic of a three-conductor, 500,000 circular mil, sector paper cable for 15,000 volt service. This cable has 0.203 inch of paper insulation on each conductor, and the radius under lead sheath is 1.11 inches, the ratio of radius noted to insulation-thickness being 5.47. Reference to Figure 4, graph of the time-factor for drying of three conductor sector paper cable possessing an impervious covering over the conductors, shows that it takes 5.5 times as long to dry a cable of this construction as it does to dry a cable with a porous conductor covering. The economic advantage of a porous construction over the impervious construction is unquestionable in this comparison.

High permeability to liquids is required to expedite impregnation. This is indicated by a capillarity test, and is discussed further below.

An electron barrier as envisaged above must necessarily be chemically inert with respect to the adjacent insulation lest the power factor or dielectric strength of the latter be injuriously affected. But mere chemical inertness is not sufficient, it being essential that this condition shall hold in the presence of electrical discharges such as may occur in voids or oil pockets within the insulation. Such discharges may result in evolution of adsorbed gas if materials which possess an adsorptive characteristic be employed; the sheet to this specification must minimize this action.

The highly capillary, porous, chemically neutral, electron barrier, subject of this invention, usually consists of between 50 and 60 percent by weight of powder supported on a residuum of fibre mesh, as described in my copending application filed February 5, 1944, Serial No. 474,885, now Patent No. 2,389,678, dated November 27, 1945.

The invention is not necessarily restricted to the three powders listed above but only a few

5 powders possess the characteristics requisite to the formation of an electron barrier sheet of this kind. They are medium density materials with a specific gravity between 3 and 6, and are special fusion products of high temperature furnaces. By virtue of their treatment in manufacture, they exhibit a marked stability of structure and are inert toward insulating fluids.

10 Metallic powders may not be employed in substitution for the above-mentioned powders, both because of their relatively low work functions and because of the deleterious effect which they have on the power factor and electrical stability of fluid insulating compound. The deleterious effect 15 on insulating compound power factor is caused by the metal oxide which coats the surface of each particle of metal powder. Aluminum, copper, iron, and other metals commonly suggested for this purpose react readily with the 20 oxygen of the atmosphere. The amount of oxide in relation to weight of metal is magnified considerably by the high degree of subdivision in powder form and consequent increase in surface area, thus accounting for the extreme vitiating 25 powers of metal powders toward fluid insulating compound.

Graphite, carbon black, and similar powders, 30 likewise, may not be used as substitutes for the higher gravity powders described above, because if used as the basic material, the resultant sheet would be mechanically weak and be characterized by a low work function. Also, it would be impossible to prevent carbon from powdering out of a sheet of this formula, unless a heavy sizing 35 were employed in the furnish. Sizing is doubly objectionable for paper of this type, first because it is extremely vitiating to fluid insulating compound, and second, because it renders the sheet impervious, thus adding the disadvantages of an 40 impervious sheet detailed above. If carbon in any form is used in small proportions as a mere modifier of paper, it is open to other objections. Thus, carbon blacks are not inert to fluids, but instead exhibit a highly developed adsorptive 45 characteristic. This would be a disadvantage in vacuum treated, fluid impregnated electric devices, since gas adsorbed by the carbon is not entirely removed by normal vacuum treatment. Therefore, it is free to be liberated later when 50 the electric device is subjected to surge voltages liable to occur under operating conditions.

The pertinent physical characteristics of a sheet made as described in my copending application are included in the following table.

55 *Physical characteristics of six mil sheet. Made from furnish beaten to a slowness of 300 cc.*

|                                         | Electron barrier sheet | Normal sheet |
|-----------------------------------------|------------------------|--------------|
| 60 Tensile strength in lbs. per sq. in. | 4,200                  | 9,000        |
| Gurley air density in seconds           | 48                     | 200          |
| Capillarity test in seconds             | Less than 1            | 70           |

65 Study of the table reveals that at the expense of slightly over 50 per cent loss in tensile strength, a loss which by no means jeopardizes the practical mechanical usefulness of the sheet, significant improvement is achieved in two characteristics which dominate the manufacturing time and operating efficiency of vacuum processed, fluid impregnated electric devices. The 70 Gurley air density for a six mil sheet is reduced from 200 to 48 seconds, which indicates that this sheet offers less than 25 per cent of the im-

pedance to gaseous fluid flow that normal sheet does. The decrease in impedance which the sheet offers to liquid impregnation is even more pronounced, being approximately one one-hundredth that of the normal sheet. Therefore, 5 this sheet may be included in the dielectric of vacuum treated, fluid impregnated electric devices, such as electric cables and condensers, without further modification of standard manufacturing procedures.

I wish it distinctly understood that my electric device with electron barrier herein described and illustrated is in the form in which I desire to make it and that changes or variations may be made as may be convenient or desirable without departing from the salient features of my invention and I therefore intend the following claims to cover such modifications as naturally fall within the lines of invention.

I claim:

1. An electric device comprising in combination a conductor, high voltage insulation therefor of the insulating oil impregnated fibrous type, an insulating oil-pervious electron barrier containing sub-microscopic silicon carbide having a 20

15

chemical formula of SiC interposed between the conductor and the insulation, whereby the insulation is protected from electric discharges from the conductor.

2. An electric device comprising in combination, a conductor, insulation therefor, said insulation impregnated with low power factor insulating fluid, an electron barrier interposed between the conductor and the insulation and applied to the surface of the insulation consisting of sub-microscopic silicon carbide having a chemical formula of SiC.

EDWIN JOSEPH MERRELL.

#### REFERENCES CITED

The following references are of record in the file of this patent:

#### UNITED STATES PATENTS

| Number       | Name     | Date          |
|--------------|----------|---------------|
| 1,814,102    | Weiset   | July 14, 1931 |
| 1,784,989    | Hill     | Dec. 16, 1930 |
| 1,084,199    | Egly     | Jan. 13, 1914 |
| 25 1,027,004 | Schwerin | May 21, 1912  |